

## UNITED STATES PATENT OFFICE

HARRY T. BENNETT AND LE ROY G. STORY, OF TULSA, OKLAHOMA, ASSIGNEES, BY DIRECT AND MESNE ASSIGNMENTS, TO MID-CONTINENT PETROLEUM CORPORATION, OF TULSA, OKLAHOMA, A CORPORATION OF DELAWARE

## METHOD OF MAKING STABLE LOW POUR POINT LUBRICATING OILS

No Drawing. Original application filed October 24, 1927, Serial No. 228,487. Divided and this application filed July 23, 1928. Serial No. 294,933. Renewed April 17, 1931.

This invention relates to methods of making stable low pour point lubricating oils. This application is a division of an application for patent on lubricating oils and methods of making the same, filed by us on Oct. 24, 1927, Serial Number 228,487, Patent Number 1,806,735, issued May 26, 1931.

One of the objects of the invention is to lower the pour point without impairing the lubricating properties of the oil.

Another object is to obtain and maintain the low pour point. In other words, this object is to produce a lubricating oil having a stable, or fixed, low pour point which is not changed by exposure to the extremes of high and low atmospheric temperatures. This object may be attained by mixing the composition at a high temperature, as will be hereafter described.

A further object is to produce a low pour point lubricating oil without causing an objectionable change in the color of the oil.

A still further object is to accomplish these results by lowering the pour point without changing the viscosity of the oil.

With the foregoing and other objects in view, the invention comprises the novel method hereinafter specifically described to set forth an embodiment of the invention.

However, it is to be understood that the invention comprehends changes, variations and modifications which come within the scope of the claims hereunto appended.

Briefly stated, we prefer to lower the pour point by adding to a lubricating oil a quantity of soap small enough to accomplish this result without materially changing the viscosity of the lubricating oil. This quantity preferably ranges between five-hundredths percent and three-tenths percent of the weight of the mass, and in actual practice we have found that one-tenth percent gives highly satisfactory results. However, as will be hereafter pointed out, there is a further problem involved in maintaining or stabilizing the low pour point. We have shown how this can be accomplished by the use of relatively high temperatures in the treatment of lubricating oils that will withstand such temperatures. A further advantage may be ob-

tained by adding a small percentage of animal oil, or vegetable oil, as will be hereafter described.

In our early efforts to lower the pour point of a paraffin base lubricating oil, without changing its viscosity, we found that the addition of very small percentages of soap, as heretofore mentioned, would produce the desired result for a more or less limited period. For example, we have prepared oils which showed pour points of  $-10^{\circ}$  F. but after exposure to weather temperatures ranging from  $+80^{\circ}$  F. to  $-20^{\circ}$  F., the pour point tended to rise and after long periods some oils even reverted to the original pour point of about  $+15^{\circ}$  F. to  $+35^{\circ}$  F. We discovered, however, that in those cases wherein the pour point was unstable, the oils had been prepared by mixing the soap in the oil at temperatures below  $300^{\circ}$  F., whereas in every case in which the soap had been mixed with the oil at temperatures in excess of  $300^{\circ}$  F. the pour point was very stable.

For the preparation of low pour point oils wherein the consistency is such that high temperatures are advantageous, or cause no serious damage, we heat the oil to temperatures preferably in excess of  $300^{\circ}$  F., for example,  $300$  to  $350^{\circ}$  F., for the step of commingling the soap in the oil.

While the oil is at a temperature between  $300$  and  $350^{\circ}$  F. we prefer to gradually mix the pure soap with the oil, and to violently agitate the mass until the mixture is uniform. In this way a stable material is obtained.

Lubricating stocks from paraffin base crudes are derived from wax distillate or that fraction of the crude coming from the still after the lower boiling point products such as gasoline, naphtha, kerosene and gas oil have been removed by fractional distillation. The wax distillate is essentially a mixture of paraffin wax and lubricating stock from which it is extremely difficult to remove a sufficient amount of wax to give a lubricant of pour point of  $0^{\circ}$  F. In our process it is not necessary to remove all of the wax from the oil, but only the major portion. We treat the remaining oil and wax mixture to produce a stable low pour point product.

A clearer understanding of our invention may be obtained by a more specific description of the details of one form of the invention.

5 A wax distillate, having a pour point of 50 to 100° F., is chilled until the major portion of the wax has separated, and the cold mixture is forced under pressure through a filter to remove the separated wax. The 10 filtered oil or pressed distillate, having a pour point of 20 to 35° F., is then separated by distillation into lubricating stocks having the same pour point and a viscosity of 90 to 1000 seconds Saybolt at 100° F., depending on 15 the grade of lubricant desired.

The lubricating stock is then bleached, by any of the well known methods of decolorization, such as the use of acid and clay, to the desired color, and the resulting lubricating oil heated to 300° to 350° F. About one-tenth percent of aluminum stearate in the form of a jell, is then thoroughly incorporated in the oil. The product has a pour point of 0 to -20° F., and is extremely stable 25 to changing temperature conditions.

In some cases it is desirable to add to the composition a small quantity of animal or vegetable oil, and we have found it advantageous to add such oils as neat's-foot oil or 30 castor oil in proportions of 2 to 10 percent of the weight of the mass, about 4 percent being preferable.

It is to be understood that we do not limit ourselves to the above example. Other soaps 35 as well as aluminum stearate, such as aluminum palmitate, zinc stearate, zinc palmitate, etc., have given good results in amounts from five-hundredths of one per cent to three-tenths of one percent.

40 Recognized procedure of determining pour points is provided in Technical Paper 323B, U. S. Government Specification No. 2d, Department of Commerce Publication, U. S. Government Master Specification for Lubricants and Liquid Fuels and Methods for 45 Sampling and Testing, on pages 40 and 41 of which is set forth Procedure for pour point.

We claim:

50 1. The method of making stable low pour point lubricating oils which consists in heating a lubricating oil composition to 300 to 350° F., and while thus heated mixing therein in five hundredths to three-tenths percent 55 soap and thereby producing a stable oil of lower pour point than the oil treated without materially affecting the viscosity thereof.

2. The method of making stable low pour point lubricating oils which consists in heating a lubricating oil composition to 300 to 350° F., and while thus heated mixing therein about one-tenth percent aluminum stearate and thereby producing a stable oil of lower 60 pour point than the oil treated without materially affecting the viscosity thereof.

3. The method of making stable low pour point lubricating oils which comprises chilling wax distillate until the major portion of the wax has crystallized, separating such portion of the wax necessary to give a dewaxed distillate of pour point 15 to 35° F., distilling said distillate to produce a lubricating stock having a viscosity of 90 to 1000 seconds Saybolt at 100° F., treating said stock to such color that temperatures herein specified cause 70 no apparent darkening, heating the oil to 300 to 350° F., and while thus heated mixing therein five-hundredths to three-tenths percent soap and thereby producing a stable oil of lower pour point than the oil treated without materially affecting the viscosity thereof.

4. The method of making stable low pour point lubricating oils which consists in chilling wax distillate until the major portion of the wax has crystallized, separating such portion of the wax necessary to give a dewaxed distillate of pour point 15 to 35° F., distilling said distillate to produce a lubricating stock having a viscosity of 90 to 1000 seconds Saybolt at 100° F., treating said stock to such 80 color that temperatures herein specified cause no apparent darkening, heating the oil to 300 to 350° F., and while thus heated mixing therein one-tenth percent aluminum stearate and thereby producing a stable oil of lower 85 pour point than the oil treated without materially affecting the viscosity thereof.

5. The method of making stable low pour point lubricating oils which consists in heating a lubricating oil of 90 to 1000 seconds Saybolt at 100° F., and containing 2 to 10 percent animal or vegetable oil to 300 to 350° F., and while thus heated mixing therein about one-tenth per cent aluminum stearate and thereby producing a stable oil of lower 95 pour point than the oil treated and without affecting the viscosity thereof.

6. The method of making a stable low pour point lubricating oil which consists in removing a portion of the wax from the oil, treating the partially dewaxed product with soap while the oil is undergoing heat treatment and thereby producing a stable low pour point oil having a lower pour point than the original oil without materially affecting the viscosity thereof.

In testimony that we claim the foregoing we hereunto affix our signatures.

HARRY T. BENNETT.  
LE ROY G. STORY.

125

130